# EUROPEAN PATENT SPECIFICATION

(11) **EP 0 604 207 B1**
(45) Date of publication and mention of the grant of the patent: **14.06.2000**
(21) Application number: 93310407.7
(22) Date of filing: 22.12.1993
(51) Int. Cl.: H01J 61/30

(54) **A metal halide arc discharge lamp**
Metall-Halogen Bogen Lampe
Lampe à arc à halogénure métallique

(30) Priority: 22.12.1992 US 995603
(43) Date of publication of application: 29.06.1994
(73) Proprietor: FLOWIL INTERNATIONAL LIGHTING (HOLDING) B.V., NL-1077 ZX Amsterdam (NL)
(72) Inventor: Jenkins, Robert G., Acton, Massachusetts 01720 (US)
(74) Representative: Butler, Michael John

(56) References cited:
- FR-A- 2 599 890
- US-A- 3 148 300
- US-A- 3 988 628
- US-A- 5 196 759

## Description

This invention relates generally to a metal halide arc discharge lamp.

Metal halide arc discharge lamps are frequently employed in commercial usage because of their high luminous efficiency and long life. A typical metal halide arc discharge lamp includes a quartz or fused silica arc tube that is hermetically sealed within a borosilicate glass lamp envelope. The arc tube, itself hermetically sealed, has tungsten electrodes mounted therein and contains a fill material including mercury, metal halide additives and a rare gas to facilitate starting. In some cases, particularly in high wattage lamps, the lamp envelope is filled with nitrogen or another inert gas at less than atmospheric pressure. In other cases, particularly in low wattage lamps, the lamp envelope is evacuated.

Sodium is an important constituent in most high intensity metal halide arc discharge lamps, usually in the form of sodium iodide or sodium bromide. Sodium is used to improve the efficiency and colour rendering properties of the metal halide lamps. It has long been recognized that sodium loss during operation is a problem with metal halide discharge lamps having arc tubes that contain sodium halides. As sodium is lost through the arc tube wall, iodide is freed and combines with mercury to form mercury iodide. Mercury iodide leads to increased reignition voltages, thereby causing starting and lamp maintenance problems.

Sodium loss results from the movement or migration of sodium ions through the arc tube wall. There are two prevailing theories relating to the cause of this sodium movement. A first theory suggests that sodium loss is caused by the emission of ultraviolet (UV) photons from the arc tube. These UV photons cause electrons to be ejected from materials, such as metals, that are positioned within the outer jacket of the lamp. The electrons ejected from these materials collect on the outside surface of the arc tube and form a negatively charged layer. The build-up of negatively charged electrons along the outer surface of the arc tube attracts positively charged sodium ions from within the arc tube and enhances their migration through the quartz arc tube wall. Once the positively charged sodium ions reach the outer surface of the arc tube wall, they are neutralized by the electrons present on the surface of the arc tube, evaporate as atoms and travel to cold spots in the lamp where they condense.

A second theory suggests that the loss of sodium from the arc tube is not primarily caused by UV radiation emitted from the arc tube. Rather, this theory suggests that the loss of sodium is due to the thermal migration of sodium ions through the arc tube wall during the operation of the lamp.

Despite the uncertainty as to its causation, sodium loss from metal halide lamps having arc tubes that contain sodium halides has long been recognized as a problem. Consequently, a number of designs have been proposed for reducing sodium loss. In a so-called "frameless construction" disclosed in US-A-3,424,935, no frame members are located close to the arc tube. By eliminating heavy metallic support rods, by using a small diameter current return wire between the lamp base and the dome end of the arc tube, and by positioning the current return wire at a relatively large distance from the arc tube, the material from which electrons can be ejected by UV radiation is greatly reduced. However, this technique for reducing sodium loss is ineffective in small low-wattage lamps.

In US-A-3,988,628 (over which claim 1 has been characterised), a thick coating of TiO₂ is fused onto the outer surface of the fused quartz arc tube. The coating of TiO₂ is reported to reduce sodium ion conductivity through the arc tube and also reduce UV radiation from the arc tube to nearly zero at wavelengths less than approximately 240nm. However, this technique for reducing sodium loss increases the cost of producing metal halide arc tube lamps because of the added expense of materials, labor and facilities needed for coating the arc tube.

In US-A-4,866,328, a coating of ZrO₂ is provided over metal surfaces positioned within the lamp envelope external to the arc tube. The ZrO₂ coating prevents UV photons from reaching the metal surfaces, thereby preventing any electrons from being ejected therefrom. In addition to ZrO₂, ceramic tubes or other ceramic coatings have also been used to perform this function. This technique of shielding the metal surfaces within the lamp envelope suffers from disadvantages in that it increases the manufacturing costs of the metal halide lamps and may not be durable for extended burn life.

It is known to utilize titanium doped fused quartz to absorb UV radiation in reprographic lamps. The reduction of UV radiation in these lamps is beneficial because at some wavelengths, the UV radiation produces ozone and at other wavelengths, the UV radiation can damage human eyesight.

From FR-A-2599890 it is known to diffuse titanium into the inner surface of a discharge lamp envelope, in particular, an envelop of a xenon discharge lamp, to prevent emission of UV radiation and to reduce internal stresses in the lamp envelope during lamp operation.

According to the present invention there is provided a metal halide lamp comprising an arc tube housed within an outer jacket, the arc tube comprising a sealed envelope and a fill material consisting substantially of mercury, metal halide additives including a sodium halide and a rare gas, characterised in that said arc tube envelope is of vitreous silica doped with between one hundred and fifty to three hundred and fifty parts per million by weight of titanium oxide.

A method for making such a lamp is defined in claim 5.

The vitreous silica may be formed by doping quartz sand with a titanium compound, such as titanium oxide, prior to melting. The preferred concentration of the titanium oxide dopant is approximately two hundred and fifty parts per million by weight. Preferred metal halide discharge lamps of the present invention utilizing arc tubes formed from the titanium oxide doped quartz can demonstrate increased lumen output and lumen maintenance.

Embodiments of the present invention will now be discussed by way of example only, and with reference to the accompanying drawings, in which:
Fig. 1 shows an example of a metal halide discharge lamp;
Figs. 2(a) - 2(d) show graphs illustrating results from a first test comparing the performance of standard production lamps with lamps having arc tubes made of quartz doped with TiO₂;
Figs. 3(a) - 3(d) show graphs illustrating the relative concentrations of various ion species as a function of time for the lamps taken over the course of the first test; and
Figs. 4(a) - 4(d) shows graphs illustrating results from a second test comparing the performance of standard production lamps with lamps having arc tubes made of quartz doped with TiO₂.

The present invention is directed to a metal halide lamp. Fig. 1 illustrates a typical metal halide arc discharge lamp in which embodiments of the present invention can be utilized. It should be understood that Fig. 1 is provided merely for illustrative purposes and that the preferred arc tubes of the present invention can be used with any type of metal halide arc tube lamp, including those having structures that differ from the example shown in Fig. 1. In Fig. 1, a lamp 2 includes a lamp envelope 4 and an arc tube 6 mounted within lamp envelope 4. The arc tube 6 is a metal halide arc discharge tube having characteristics that are described below.

The arc tube 6 is supported within the envelope 4 via a lower support means 8 and an upper support means 10. Lower support means 8 comprises a U-shaped support made up of vertical wires 14 and 16 extending from a base wire 18. The vertical wires 14 and 16 are welded to a strap 20 that supports the lower end of the arc tube 6. Upper support means 10 similarly comprises a U-shaped support made up of vertical wires 22 and 24 extending from a base wire 26. The vertical wires 22 and 24 are welded to a strap 28 that supports the upper end of the arc tube 6.

Electrical energy is coupled to the arc tube 6 through a base 28. A pair of stiff lead-in wires 30 and 32 are electrically connected to the base 28. Lead-in wire 32 is welded to base wire 18 of the lower support means 8. An additional lead-in wire 34 is electrically connected to vertical wire 16 of lower support means 8. Lead-in wire 34 is connected, via a molybdenum foil 36, to an electrode 38 within the arc tube 6. A resistor 40 is attached to lead-in wire 30 and to a connector 42. Connector 42 is connected, via a molybdenum foil 44, to a starting probe 46.

At the upper end of arc tube 6, a lead-in wire 48 is attached, via a molybdenum foil 50, to an electrode 52. Lead-in wire 48 is electrically connected to stiff lead-in wire 30 through a thin conducting lead 54. The molybdenum foils 36, 44 and 50 are located in press seals at opposite ends of arc tube 6.

As stated above, the present invention is directed to improving an arc tube for use in a metal halide lamp such as the one shown in Fig. 1. The arc tube of the present invention is formed of a titanium oxide doped vitreous silica. In one embodiment of the invention, the vitreous silica is fused quartz that is made from a melt doped with TiO₂. This doped quartz is hereafter referred to as "ozone free quartz" because the titanium oxide dopant reduces the emission of UV radiation from the arc tube that would produce ozone. By utilizing ozone free quartz rather than conventional quartz in forming the arc tube, it is believed that sodium loss from the arc tube is reduced in two ways. First, the titanium oxide in the ozone free quartz may help to retard the movement of sodium ions through the arc tube wall. Second, the titanium oxide in the ozone free quartz absorbs UV radiation so that the amount of UV radiation emitted from the arc tube is reduced. As previously stated, one theory regarding the cause of sodium loss in metal halide lamps suggests that UV photons emitted from the arc tube cause electrons to be ejected from materials in the outer jacket, thereby generating a negatively charged layer that attracts positively charged sodium ions through the arc tube wall. Consequently, by reducing the amount of UV radiation emitted from the arc tube, it is believed that the use of ozone free quartz results in a reduction of sodium loss from the arc tube of the metal halide discharge lamp.

In order to verify the performance of the arc tubes made from ozone free quartz, a series of tests was run comparing four standard production GTE M175U Metalarc lamps (utilizing arc tubes made from quartz that did not contain a TiO₂ dopant), with four GTE M175U Metalarc lamps having arc tubes made of ozone free quartz. All the test lamps were made at the same time as part of a single production run. The ozone free quartz was made by doping the quartz sand normally utilized to form metal halide arc tubes with TiO₂ prior to melting. Thereafter, the mixture of quartz sand and TiO₂ was melted and formed into arc tubes in a conventional manner that is known to those skilled in the art.

The concentration of titanium oxide in the ozone free quartz utilized for the test run described above was 250 parts per million by weight. However, it is believed that the advantages of the present invention can be achieved with ozone free quartz having various other concentrations of titanium oxide within the range of 150 to 350 parts per million by weight. Additionally, although TiO₂ was used as the dopant in forming the ozone free quartz, other titanium compounds could also be utilized that form titanium oxide when heated. Examples of other titanium compounds that are believed to be suitable for use as a dopant are titanium nitrate and compounds from the family of titanium alkoxides, such as tetrabutyl titanate. Similarly, although the arc tubes utilized in the test lamps were formed from doped quartz, it should be appreciated that arc tubes embodying the present invention can also be formed from other types of vitreous silica such as synthetic silica produced from silane.

Prior to forming the ozone free quartz into tubes, it was vacuum baked to a low hydroxyl content indicated by a Beta_{OH} of 0.0005 to 0.0007 nm⁻¹. Testing indicated that the amount of UV radiation emitted from the ozone free quartz was reduced to approximately zero at wavelengths below approximately 200 nm, with the 50% UV cut-off at approximately 240 nm. This test verifies that the use of ozone free quartz should successfully reduce the UV radiation emitted from the arc tube. As a result, the amount of photons available for ejecting electrons from materials in the outer jacket should be significantly reduced, thereby reducing sodium loss in comparison to metal halide lamps having arc tubes formed from conventional fused quartz.

Figs. 2(a) - 2(d) show a comparison of the results of a first test comparing the performance of the four lamps having ozone free quartz arc tubes (indicated by plots 30, 32, 34 and 36) with the four standard production lamps (indicated by plots 31, 33, 35 and 37). Figs. 2(a)-2(d) are graphs of arc tube voltage, lumen output, colour temperature and colour rendering index, respectively, as a function of time. As can be seen from Fig. 2(b), the lamps having arc tubes made from ozone free quartz (indicated by plot 32) displayed roughly a 20% improvement in both lumen output and lumen maintenance at 6,000 hours from the standard production lamps (indicated by plot 33). The improvement in lumen output and lumen maintenance indicates that lamps utilizing ozone free quartz arc tubes have a significant performance advantage over lamps with arc tubes made from conventional fused quartz.

The improvement in both lumen output and lumen maintenance was unexpected prior to conducting the above-described test. The reason for the improved lumen output and lumen maintenance exhibited by the arc tubes made from ozone free quartz is not precisely known. It is possible that the increased sodium retention resulting from the use of the titanium oxide dopant enables the arc tubes made from ozone free quartz to have greater lumen output over a longer period of time than conventional arc tubes. It is also possible that the titanium oxide dopant changes the conductivity of the arc tube, thereby altering the energy balance in a manner that results in the generation of an increased amount of visible radiation. Additionally, the energy balance may also be altered by the conversion of UV radiation into thermal or visible radiation since the titanium oxide dopant inhibits UV radiation from escaping the arc tube.

An analysis of Figs. 2(a) - 2(d) demonstrates that the lamps having arc tubes made from ozone free quartz not only demonstrated improved lumen output and lumen maintenance, but also did not demonstrate any significant deficiencies with regard to other lamp characteristics. Although the lamps made with arc tubes of ozone free quartz had a higher voltage rating, their voltage reached a plateau at approximately 3,000 hours and thereafter remained steady while the voltage of the standard production lamps continued to rise in an undesirable fashion. The colour rendering index (CRI) remained lower for the lamps utilizing the ozone free quartz arc tubes for the majority of the test. The voltage plateau and lower colour rendering index for the lamps having ozone free quartz arc tubes is believed to be the result of a reduction in sodium loss from those arc tubes.

Figs. 3(a) - 3(d) are graphs showing the relative concentrations of various ion species as a function of time for the lamps having arc tubes made from ozone free quartz (indicated by plots 38, 40, 42 and 44) and the standard production lamps (indicated by plots 39, 41, 43 and 45). These graphs show no major differences in the arc species contents between the groups, although the iodine content of the ozone free group (indicated by plot 44) hit a plateau early while that of the control group (indicated by plot 45) gradually dropped. The similarity of values for scandium and sodium in the two groups of lamps suggests that the higher lumen production in the group of lamps with the ozone free quartz arc tubes did not result from heating of those arc tubes.

Figs. 4(a) - 4(d) illustrate the results of a second lamp test which utilized double ended lamps of a nonstandard design. The control group (indicated by plots 47, 49, 51 and 53) utilized standard 175W production arc tubes while the test group (indicated by plots 46, 48, 50 and 52) utilized lamps that were made at the same time and were identical except for the use of arc tubes formed from ozone free quartz. Many of the lamps in both groups failed early in the test as a result of oxidation at the inleads of the outer jacket. However, those that survived showed that the lamps with the ozone free arc tubes again had higher lumen output and lumen maintenance than the lamps with the conventional quartz arc tubes. These results are consistent with the results of the first test shown in Figs. 2(a) - 2(d). Each of these tests indicates that lamps having arc tubes made from ozone free quartz perform significantly better in terms of both lumen output and lumen maintenance than lamps utilizing conventional arc tubes.

Embodiments of the present invention may provide an arc discharge lamp wherein sodium loss from the arc tube is relatively low; and further may provide a metal halide discharge lamp having increased light output.

## Claims

1. A metal halide lamp comprising an arc tube housed within an outer jacket, the arc tube comprising a sealed envelope (6) and a fill material consisting substantially of mercury, metal halide additives including a sodium halide and a rare gas, characterised in that said arc tube envelope (6) is of vitreous silica doped with between 150 to 350 parts per million by weight of titanium oxide.

2. A metal halide lamp as claimed in claim 1, wherein the concentration of titanium oxide in the vitreous silica is about 250 parts per million by weight.

3. A metal halide lamp as claimed in claim 1 or 2, wherein the vitreous silica comprises fused quartz.

4. A metal halide lamp as claimed in any of claims 1, 2 or 3, wherein said lamp further comprises an arc tube support assembly (8,10) and means (28,30,32 etc.) for coupling electrical energy to said arc tube.

5. A method of making a metal halide lamp as claimed in any of claims 1 to 4, characterised in that the envelope (6) for the arc tube is made by adding a titanium compound to the raw materials at a melt stage such that vitreous silica doped with titanium oxide is produced for forming said envelope.

6. A method as claimed in claim 5, wherein the titanium compound is titanium oxide.

7. A method as claimed in claim 5, wherein the titanium compound forms titanium oxide when heated.

## Patentansprüche

1. Metallhalogenidlampe mit einem in einer äußeren Ummantelung angeordneten Brenner, welcher eine abgedichtete Hülle (6) und ein Füllmaterial aufweist, das im wesentlichen Quecksilber und Metallhalogenidadditive mit Natriumhalogenid und einem Edelgas umfaßt, dadurch **gekennzeichnet**, daß die Hülle (6) des Brenners aus Quarzglas besteht, das mit zwischen 150 bis 350 Gewichts-ppm Titanoxid datiert ist.

2. Metallhalogenidlampe nach Anspruch 1, bei welcher die Titanoxidkonzentration in dem Quarzglas etwa 250 Gewichts-ppm beträgt.

3. Metallhalogenidlampe nach Anspruch 1 oder 2, bei welcher das Quarzglas aus geschmolzenem Quarz besteht.

4. Metallhalogenidlampe nach einem der Ansprüche 1, 2 oder 3, bei welcher die Lampe außerdem einen Brennerhalterungsaufbau (8, 10) und Elemente (28, 30, 32 etc.) für den Anschluß von elektrischer Energie an den Brenner aufweist.

5. Verfahren zur Herstellung einer Metallhalogenidlampe nach irgendeinem der Ansprüche 1 bis 4, dadurch **gekennzeichnet**, daß die Hülle (6) für den Brenner durch Hinzufügung einer Titaniumverbindung zu den Rohmaterialien im Schmelzzustand hergestellt wird, derart, daß mit Titaniumoxid datiertes Quarzglas für die Ausbildung der Hülle erzeugt wird.

6. Verfahren nach Anspruch 5, bei welchem die Titaniumverbindung Titaniumoxid ist.

7. Verfahren nach Anspruch 5, dadurch **gekennzeichnet**, daß die Titaniumverbindung Titaniumoxid bildet, sobald sie aufgeheizt wird.

## Revendications

1. Lampe à halogénures métalliques comprenant un tube à arc logé à l'intérieur d'une chemise extérieure, le tube à arc comportant une ampoule scellée (6) et un matériau de remplissage comprenant substantiellement du mercure, des additifs d'halogénures métalliques incluant un halogénure de sodium et un gaz rare,
**caractérisée en ce que**
la dite ampoule (6) du tube à arc est en silice vitreuse dopée avec entre 150 et 350 parts par million en poids d'oxyde de titane.

2. Lampe à halogénures métalliques selon la revendication 1, dans laquelle la concentration d'oxyde de titane dans la silice vitreuse est de 250 parts environ par million en poids.

3. Lampe à halogénures métalliques selon la revendication 1 ou 2, dans laquelle la silice vitreuse est du quartz fondu.

4. Lampe à halogénures métalliques selon l'une quelconque des revendications 1, 2 ou 3, dans laquelle la dite lampe comprend, en outre, un ensemble de support (8, 10) du tube à arc et des moyens (28, 30, 32, etc...) pour appliquer l'énergie au dit tube à arc.

5. Procédé de fabrication d'une lampe à halogénures métalliques selon l'une quelconque des revendications 1 à 4, caractérisé en ce que l'ampoule (6) du tube à arc est réalisée en ajoutant un composé de titane aux matériaux bruts lors d'une étape de fusion, de telle façon que la silice vitreuse dopée avec de l'oxyde de titane soit obtenue pour former la dite ampoule.

6. Procédé selon la revendication 5, dans lequel le composé de titane est de l'oxyde de titane.

7. Procédé selon la revendication 5, dans lequel le composé de titane forme de l'oxyde de titane lorsqu'il est chauffé.
